

# UNITED STATES PATENT OFFICE.

WALTER O. SNELLING, OF ALLENTOWN, PENNSYLVANIA, ASSIGNOR TO TROJAN POWDER COMPANY, OF NEW YORK, N. Y., A CORPORATION OF NEW YORK.

## METHOD OF TREATING UNDRIED ORGANIC NITRATES AND THE LIKE.

1,386,439.

Specification of Letters Patent.

Patented Aug. 2, 1921.

No Drawing. Application filed March 16, 1920, Serial No. 366,390. Renewed January 21, 1921. Serial No. 439,054.

*To all whom it may concern:*

Be it known that I, WALTER O. SNELLING, a citizen of the United States, and resident of Allentown, Lehigh county, Pennsylvania, 5 have invented certain Improvements in the Method of Treating Undried Organic Nitrates and the like, of which the following is a specification.

My invention relates to the manufacture 10 of explosives and similar materials which, owing to the manufacturing processes employed, are obtained in wet condition, and the object of the invention is to provide a method for reducing the water content of 15 such materials without drying. While my invention may be utilized in the manufacture of a number of materials, I have found it particularly useful as applied to the manufacture of explosives, and for purposes of 20 specific illustration will describe it in connection with such manufacture.

In the manufacture of nitrocellulose, nitrostarch and other solid organic nitrates, said materials, following the nitration and 25 washing processes, are in wet condition, and it has hitherto been the practice to dry them before mixing with other ingredients to produce commercial or military explosives. Even where it has been desired to produce 30 a wet finished explosive, the preliminary drying process has been deemed necessary because of the undue amount of water present with the organic nitrate following the washing process. While it is manifestly de- 35 sirable to avoid the drying operation by utilizing the nitrostarch or nitrocellulose in wet condition, as in this way an important item of expense and danger is avoided, experiments have shown that explosives of 40 proper sensitiveness cannot be made by the mere mixing of salts with undried nitrostarch or nitrocellulose. For example, nitrostarch after coming from the centrifuge and having its water content reduced there- 45 in to the lowest obtainable amount, still contains an average of about 20% of moisture. If now such wet nitrostarch is mixed in equal parts with nitrate of soda or with nitrate of ammonia the completed mix will 50 still contain 10% of moisture, and this is higher than the amount which such a mix can contain and still detonate with such detonating caps as are commercially used. It is true that by using a smaller amount of

the wet nitrostarch, and a greater amount 55 of the nitrate, mixtures having a lower water content can be obtained. One part of wet nitrostarch may for example be mixed with three parts of sodium nitrate, and in this case if the initial nitrostarch contained 60 20% of water the final mix will contain but 5% of water. Such a mix is, however, quite as insensitive as the mixture previously described, and which contained 10% of water, 65 for the reason that the amount of nitrostarch has been reduced in proportion as the water has been reduced, the first mixture containing 40% of nitrostarch on a dry basis, and 10% of water, and the second mixture containing 20% of nitrostarch on a dry 70 basis, and 5% of water, and both of these mixtures being insensitive to detonation.

Repeated experiments have shown that there are no proportions in which wet nitrostarch or wet nitrocellulose, after drying to 75 the maximum extent possible in a centrifugal wringer, can be mixed with nitrate of soda or with nitrate of ammonia to form an explosive susceptible to detonation with the No. 6 or No. 7 detonators commonly 80 used in commercial work.

I have discovered an inexpensive and convenient method by which sensitive explosives may be obtained from organic nitrates without recourse to the normal drying operation. As an example of my invention, I will describe the method by which I make a nitrostarch explosive from nitrostarch containing 25% of water. 85

I first prepare a concentrated solution of 90 ammonium nitrate and water, preferably using a solution containing about 65% of dissolved ammonium nitrate. I thoroughly mix my wet nitrostarch with such a solution, either by mixing the wet nitrostarch 95 with the solution and then applying centrifugal force to remove the excess, or by an operation of displacement. In any case I substitute a solution of ammonium nitrate for the water which is normally present 100 in the wet material.

As the result of this first stage of my procedure, I obtain instead of nitrostarch wet with 25% of water, nitrostarch which contains 25% of a concentrated solution of ammonium nitrate. As the water originally present in the nitrostarch tends to dilute my original ammonium nitrate solution, in or- 105

dinary procedure I obtain an absorbed solution containing about 50% by weight of ammonium nitrate, and my nitrostarch contains about 25% by weight of this solution, 5 after moderate wringing.

If I now mix equal weights of the nitrostarch so prepared with ammonium nitrate, I obtain a mixture which contains 37.5% of nitrostarch, 56.25% of ammonium nitrate, 10 and 6.25% of water. This mixture is sensitive to commercial detonators, and forms a highly desirable explosive. I may employ 70% of my wet nitrostarch and 30% of ammonium nitrate, and in this case my finished 15 explosive contains 52.5% of nitrostarch, 38.75% of ammonium nitrate, and 8.75% of water, this explosive also being sensitive to a commercial detonating cap.

Through treatment as described, my ammonium nitrate solution becomes diluted through 20 the water taken up from the nitrostarch, and becomes impoverished through the giving up to the nitrostarch of part of its dissolved ammonium nitrate. Accordingly I may from 25 time to time add more ammonium nitrate, and I may if necessary remove portions of the liquid from time to time and concentrate same. Preferably I so adjust the moisture in 30 my nitrated product that the amount of dissolved inorganic nitrate taken up by the nitrostarch or the nitrocellulose balances as nearly as possible the amount of water given up to the bath.

From the foregoing illustration it will be 35 seen that while the liquid content of the explosive material is not reduced, the water content has been reduced, a portion of the latter being replaced by an ingredient having a function in the finishing explosive. 40 Obviously other inorganic oxidizing salts having a high solubility in water may be substituted for ammonium nitrate, such, for example, as calcium nitrate, or ammonium or sodium chlorate or perchlorate. In the 45 manufacture of some explosives, or other material, the displacing solution need not necessarily be that of a salt performing any function in the finished product other than the displacing function, the method in its 50 broader aspect contemplating the reduction of the water or other liquid content of a wet material by replacement by a concentrated solution of an inorganic salt.

The solid salt which is admixed with the 55 wet organic nitrate prepared as described in

this application may or may not be the same material of which a solution is used for displacing the water originally present in the organic nitrate. For example, the water originally present in undried nitrated starch 60 may be displaced by means of a concentrated solution of ammonium nitrate, and the wet nitrostarch so prepared may then be mixed with dry ammonium nitrate or the nitrated starch prepared as described may be mixed 65 with dry sodium nitrate, or with dry ammonium perchlorate or with any other suitable dry salt or mixture of dry salts. Instead of a solution of ammonium nitrate or other inorganic salt I may use a concentrated solution 70 of any solid body having high solubility in water.

I claim:

1. The method of treating wet materials to reduce the water content without drying 75 which comprises the step of replacing a portion of said water by a concentrated solution of a solid body having high solubility in water.

2. In the method of manufacturing explosives and the like containing a solid organic nitrate, the step which comprises displacing water present in the undried organic nitrate by a concentrated solution of an inorganic nitrate. 80

3. The method of manufacturing wet explosives containing an organic nitrate and an inorganic salt which comprises the step of displacing water originally associated with said organic nitrate by a solution of 85 said inorganic salt.

4. The process of making a wet explosive containing a solid organic nitrate and an inorganic salt without drying said organic nitrate, which comprises reducing the amount 95 of water content in said organic nitrate to a required amount by the substitution of a solution of said inorganic salt and thereafter adding sufficient of the dry inorganic salt to secure the desired proportion of the several 100 ingredients.

5. In the manufacture of explosives, the process which comprises displacing a part of the water present in a wet organic nitrate by means of a concentrated solution of a 105 solid body having high solubility in water, and admixing the product so obtained with inorganic oxidizing agents.

WALTER O. SNELLING.